

May 10, 1949.

A. J. WEINIG

2,469,422

SELECTIVE FLOTATION OF CHROMITE ORES

Filed Dec. 20, 1943



ARTHUR J. WEINIG  
INVENTOR.

BY

*H. A. McGraw*  
ATTORNEY

## UNITED STATES PATENT OFFICE

2,469,422

## SELECTIVE FLOTATION OF CHROMITE ORES

Arthur J. Weinig, Golden, Colo.

Application December 20, 1943, Serial No. 514,987

4 Claims. (Cl. 209—167)

1

This invention relates to a froth flotation treatment of chromite ores, and more particularly relates to the treatment of chromite beach sands, or the treatment of the product of a gravity concentration of such beach sands.

Deposits of the aforesaid character occur in a variety of places. As an example, chromite beach sands of Coos County, Oregon have been found to be particularly amenable to the present treatment. A variety of minerals are contained in such sands, as for example, chrome, spinels, zircon, staurolite, ilmenite, magnetite, garnet as well as a quartz, epidote, olivine and its alteration products.

In the case of beach sands the chromite content is rather small, the aforesaid Coos County, Oregon sands having a  $\text{Cr}_2\text{O}_3$  content of about 6%. Due to long weathering and exposure, the mineral surfaces have been altered to such an extent that the material will not respond to conventional froth flotation treatments. Further, because of the low chrome content expensive processing is not feasible for commercial operations.

It is an object of the present invention to provide a simple, efficient and economical froth flotation process for the treatment of chromite ores providing a selective recovery of the chromite and/or other valuable constituents of the ores.

Another object of the invention is to provide a froth flotation treatment of chromite ores in which the solution of the pulp may be recovered and recirculated through the treatment stage in which it initially was used.

A further object of the invention is to provide a novel procedure for the apportioning of the reagent ingredients used in a froth flotation treatment of chromite ores.

Other objects of the invention include novel steps and treatments, all of which will be fully described in the course of the following description.

Briefly stated, the invention comprises an initial bulk flotation filming of the constituent minerals in the presence of a fluosilicate-forming composition, partially neutralizing the resulting acidified surfaces to a degree which will permit flotation collectors to produce flotation, and then partially acidifying again to promote selective flotation of different minerals of the composition. When so conditioned, the selected minerals of the pulp will respond readily to the action of a fatty acid collector under the influence of aeration and carry to the surface in a froth where they may be removed by overflow.

In order to effectively acidify and neutralize

2

the particle surfaces, particularly when a continuous operation is employed, an exact test procedure has been developed for use in performing the flotation process. This procedure will be best understood by describing a typical test operation treating a gravity concentrate of Coos County, Oregon, beach sands.

1500 ml. water and 0.5 gram of sodium silicofluoride were introduced into a 500 gram mechanical laboratory flotation machine. This composition was agitated and then 25 ml. of the mixture was titrated with a caustic soda solution (equivalent to 8.66 gr. oxalic acid per litre). The ml. used multiplied by 0.4 will indicate the equivalent acidity in pounds of  $\text{Ca}(\text{OH})_2$  per ton of solution. This should be around .4 lb.

 $\text{Ca}(\text{OH})_2$ 

per ton of solution.

20 750 to 1000 grams of a gravity concentrated chrome ore at 48 mesh and containing about 25%  $\text{Cr}_2\text{O}_3$  was introduced into the above solution and agitated or blunged for fifteen minutes with no aerating gas introduced. When agitation was stopped 25 ml. of the upper solution was drawn off, a phenol indicator added, and titrated with the caustic soda solution. Only a slight drop in the titration should be noted, probably not below .36  $\text{Ca}(\text{OH})_2$  per ton of solution.

25 30 Thereafter, the following reagents were introduced into the conditioned pulp in the amounts and orders stated:

- 35 1. .6 ml. 30% aqueous solution of caustic soda (300 grams per litre) about 7.5 normal.
2. 10 drops gas oil or crude kerosene.
3. 10 drops of petroleum aliphatic acid (Standard Oil Co. of California No. 30395-R).
4. 20 ml. of a 5% solution formed by treating 50 ml. distilled talloel with 20 ml. ammonia sol. (25 Bé.) and diluting with 1000 c. c. water.

40 After so introducing the reagents into the pulp, it was agitated for from three to five minutes. Next the solution was tested by titration, which must indicate between .16 and .08 lb.  $\text{Ca}(\text{OH})_2$  per ton of solution. The pulp was then diluted to a suitable flotation volume, adding 1 ml. aqueous sulfuric acid solution (equivalent to 30% aqueous solution of caustic soda).

45 50 After this conditioning, the air was turned on and the froth skimmed off after aerating for one to two minutes. The machine then was emptied, the liquid decanted and the separated solution saved. The reject tailings of this separation were quartz, epidote, olivine and alteration products together with some garnet.

Next, the froth concentrate was returned to the machine, mixed with the decanted solution, agitated for two minutes, after which 2 ml. aqueous sulfuric acid solution was added. The air was turned on and the froth concentrate removed after aerating one to two minutes. The residue again was decanted, and the tailings, in this case clear garnet, were removed.

Following this two stage separation, a third separation was made to produce a higher grade 10 chromite concentration. The froth concentrate of the preceding separation was returned to the machine, mixed with the decanted solution with 1 ml. aqueous sulfuric acid solution and 15 ml. of 5% quebracho extract added and then re-floated.

The tailings of this treatment include additional varieties of garnet, zircon, magnetite, ilmenite and chrome spinels, staurolite etc., which should be classed as a middling. Titration of 20 the solution of this operation should end in a blue reaction color instead of a pink. The titration should be about .6 to .7.

With this understanding of the operating procedure to be followed in the practice of the present invention, some typical tests will be cited to illustrate the efficiency of the treatment. In the first of these, the ore taken for test was a gravity concentrated beach sand which assayed 26.5% Cr<sub>2</sub>O<sub>3</sub>. The treatment performed was a 30 substantial duplicate of that enumerated hereinbefore. The results follow:

#### Test 1

| Product          | Wt. | Percent Wt. | Percent Cr <sub>2</sub> O <sub>3</sub> | Percent Recovery |
|------------------|-----|-------------|----------------------------------------|------------------|
| Concentrate..... | 475 | 62.3        | 40.7                                   | 99               |
| Tails.....       | 275 | 36.7        | 0.7                                    |                  |
| Total.....       | 750 |             |                                        |                  |

A similar treatment of another ore sample of gravity concentrated beach sand assaying 28% Cr<sub>2</sub>O<sub>3</sub> was undertaken and the results follow:

#### Test 2

| Product          | Wt.   | Percent Wt. | Percent Cr <sub>2</sub> O <sub>3</sub> | Percent Recovery |
|------------------|-------|-------------|----------------------------------------|------------------|
| Concentrate..... | 650   | 65.0        | 41.8                                   | 97.5             |
| Tails.....       | 350   | 35.0        | 1.0                                    |                  |
| Total.....       | 1,000 |             |                                        |                  |

A third test was undertaken with additional ore from the same sample as used for Test 2. The results of the treatment follow:

#### Test 3

| Product          | Wt. | Percent Wt. | Analyses                               |             |                          | Percent Recovery |
|------------------|-----|-------------|----------------------------------------|-------------|--------------------------|------------------|
|                  |     |             | Percent Cr <sub>2</sub> O <sub>3</sub> | Percent FeO | Percent TiO <sub>2</sub> |                  |
| Concentrate..... | 455 | 57          | 45.4                                   | 26.75       | 1.9                      | 92               |
| Tails.....       | 295 | 43          | 5.35                                   |             |                          |                  |
| Total.....       | 750 |             |                                        |             |                          |                  |

The rougher tailings of the first stage flotation 70 separation was 6% by weight and analyzed 1% Cr<sub>2</sub>O<sub>3</sub>. The product from the second flotation stage was 32% by weight and analyzed .6 of 1% Cr<sub>2</sub>O<sub>3</sub>. The tailings from the final flotation stage was 5% by weight and analyzed 32½% Cr<sub>2</sub>O<sub>3</sub>.

The final concentrate was 57% by weight and analyzed 45.4 Cr<sub>2</sub>O<sub>3</sub>.

The concentrate made in this test was subjected to fractional magnetic separation with the following results:

| Product        | Percent Wt. | Cr <sub>2</sub> O <sub>3</sub> | FeO   | TiO <sub>2</sub>                 |
|----------------|-------------|--------------------------------|-------|----------------------------------|
| 0.2 Amp. Conc. | 1.6         | 10.54                          | 50.97 |                                  |
| 1.7 Amp. Conc. | 6.0         | 15.90                          | 46.06 | 25.76.                           |
| 3.0 Amp. Conc. | 4.4         | 31.10                          | 33.71 | (1) About 10% garnet.            |
| 5.0 Amp. Conc. | 84.7        | 50.25                          | 24.96 | (2) About 1½% silicate minerals. |
| Residue.....   | 3.3         |                                |       | (3) Mostly zircon.               |

A study of these magnetic fractions leads us to conclude that a chrome concentrate of about 52% Cr<sub>2</sub>O<sub>3</sub> grade is the ultimate which can be made. Aside from the evident magnetite and ilmenite present there are chrome spinels present of various Cr<sub>2</sub>O<sub>3</sub> content and these minerals must be dropped out to attain maximum grade at the expense of recovery.

From the foregoing, it will be apparent that by subjecting a pulp, inclusive of concentrates from a preceding operation, to a succession of flotation actions with an increase in acidity at each successive stage, it is possible to reject minerals of the pulp until only a purified chromite is collected as froth concentrate.

In the aforesaid tests, the treatment procedure has involved batch methods, but it will be apparent that the process can be performed effectively as a continuous operation. In such a treatment, conditioning tanks will be placed ahead of each flotation section and the required conditioning interval can be maintained at each stage. Also, once the requirements of a given operation are known, the acidity changes can be closely regulated with periodic reagent introduction at each conditioning stage.

Where the liquid of the pulp is to be recirculated, it will be desirable because of the acidity regulation to only introduce such liquid into whatever flotation battery it has been withdrawn from. To do otherwise would upset the acidity controls, which are quite important in obtaining the desired selective action. A convenient means for dewatering the pulp after collection of the concentrate at a given stage is to direct the tailings discharge into a mechanical type classifier. The various sands are relatively heavy and settle quite easily, so that a substantially clear liquid is passed across the overflow of the classifier and the raked product can be removed as a reject material or collected as a market product according to its composition and market value.

A variety of reagent compositions have been tested and numerous substitute materials have been found to be suitable for use in the process. In the initial blunting treatment a number of compositions have given good results. I have described the use of sodium silico fluoride, and, in

addition, various laundry sours or fluoride sours, such as sodium bifluoride, sodium fluoride and hydrofluoric acid may be used. These various fluosilicate-forming ingredients serve to condition the material for a bulk flotation action, after which by neutralizing to a degree where only quartz, epidote, olivine and alteration products will be rejected a concentrate is produced by froth floating in the presence of a fatty acid collector. In this action, I prefer to use an oil such as crude kerosene or gas oil to promote the filming. Almost any fatty acid soap will function as a collector reagent if the proper acid conditions for such soap are established in the treatment. I preferably use a fatty acid with three double bonds such as an ammonium salt of linoleic or ammonium linoleate. Beneficial results are derived if a frother is used, and petroleum aliphatic acids, steam distilled pine oil or cresylic acid may be used for this purpose.

In operations where a high degree of selectivity is desired, I introduce into the final flotation stage an additional reagent such as a 5% quebracho extract or lignin, tannic acid or its derivatives, and thereby impede the flotation of all minerals except the chromite. Due to the stage flotation treatment employed and the elimination of constituent minerals at each stage, it will be apparent that a substantial amount of the  $\text{Cr}_2\text{O}_3$  content will be eliminated by such procedure. The final product is a purified chromite containing very little material that may be classed as contaminant, but whenever such a purified product is not required, the recovery can be raised by reducing the selectivity of the treatment.

The accompanying flowsheet illustrates a typical circuit used in the practice of the present invention. As illustrated, a conditioner tank 1 is supplied with a suitable chromite ore pulp introduced at 2 while sodium silico-fluoride is fed in at 3 to produce an acidity condition in the pulp equivalent to .40 lb.  $\text{Ca}(\text{OH})_2$  per ton of solution. When so conditioned the pulp is discharged at 4 into a second conditioning tank 5 in which a mixture of caustic soda, kerosene, petroleum aliphatic acid frother and ammonia talcool mixture are fed to the pulp at 6 to produce an acidity equivalent to .08 to .16 lb.  $\text{Ca}(\text{OH})_2$  per ton of solution.

The pulp so conditioned is discharged at 7 into a flotation cell or stage where enough mineral acid, preferably sulfuric acid, is introduced at 9 to bring the acidity of the pulp within the equivalent range of from .03 to .05 lb. per ton of  $\text{Ca}(\text{OH})_2$  per ton of solution. A bulk flotation of the chromite is obtained in cell 8 with the reject material consisting of quartz, epidote, olivine and alteration products being discharged at 10 while the collected froth is overflowed at 11. The tailings pass into a thickener 12 with the sludge discharge 14 thereof passing to waste while the clarified liquid is drawn from the thickener overflow 13 and passes to a second flotation stage 15 in which the froth overflow from 11 also is introduced together with additional sulfuric acid as indicated at 16 to produce a pulp acidity equivalent to .50 lb.  $\text{Ca}(\text{OH})_2$  per ton of solution. The collected froth concentrate is removed by overflow at 17 and the reject tailings pass through a line 18 into a thickener 19 from which the sludge discharge of which garnet is the principal constituent may be collected as a concentrate.

The clarified liquid collected in thickener 19 passes through a line 21 to another flotation

stage 22 in which the froth concentrate from 17 is delivered and in which additional mineral acid is introduced as at 23 to produce a pulp acidity equivalent to .55 lb.  $\text{Ca}(\text{OH})_2$  per ton of solution. The tailings reject of this stage, consisting principally of middlings, is discharged at 24 and may be and preferably is returned to the initial flotation stage 8 while the froth concentrate is overflowed at 25 and passes into another flotation stage 26. A quantity of quebracho extract is introduced into this pulp which by further acidity control is maintained at an acidity equivalent to .65 lb.  $\text{Ca}(\text{OH})_2$  per ton of solution. The collected froth is discharged at 28 as the final chrome concentrate, while the tailings reject consisting of various chrome-containing minerals may be taken on to further treatment, if desired, or may be handled as a bulk concentrate.

The flow sheet just described is particularly suited for the performance of the present process in continuous operation. However, it should be understood that variations in the circuit are intended to suit commercial requirements. Thus, if the rejection of quartz, olivine, epidote and the like with the tailings at flotation stage 8 produces a market grade concentrate, it may be necessary to follow with only one additional flotation treatment to separate garnet from chrome and obtain the final market products. Also in batch operations a single flotation stage may be adequate, and by selective acidity control a plurality of final products may be obtained.

I have described the treatment of Oregon beach sands, but it will be understood that the same treatment procedure with proper readjustment may be followed with equally good results in treating mined chromite ores. Where freshly mined ores are taken for treatment, the initial blunging treatment may be shortened or eliminated if there are no altered surfaces that have to be acted upon, and preferably such a blunging treatment will follow the grinding stage of the treatment. Where closed circuit grinding is practiced, the classifier overflow may be conducted to suitable agitating or conditioning apparatus in which the laundry sours will be introduced.

The flotation treatments may be performed in suitable froth flotation apparatus, and preferably in mechanical type flotation machines. The treatment interval is of relatively short duration as the mineral floats quite readily after the conditioning hereinbefore described.

Changes and modifications may be availed of within the spirit and scope of the invention as defined in the hereunto appended claims.

What I claim and desire to secure by Letters Patent is:

1. A selective froth flotation process for the treatment of chromite ores having low grade chrome spinels, zircon, staurolite, ilmenite, magnetite, garnet, quartz, epidote, olivine and alteration products as inclusions, which comprises subjecting a pulp of such an ore to an initial blunging treatment in the presence of a soluble fluosilicate-forming substance, partially neutralizing the acidified particle surfaces by introducing a caustic into the pulp, subjecting said pulp to a bulk froth flotation action in the presence of a fatty acid collector to concentrate the chrome-containing constituents of the pulp, refloating the concentrate of the treatment in a plurality of cleaning actions while increasing the acidity of the pulp in each such refloating

action through the introduction of a mineral acid therein, whereby to selectively reject different minerals of the pulp, and recovering a purified chromite concentrate as a final product of the treatment.

2. A selective froth flotation process for the treatment of chromite ores having low grade chrome spinels, zircon, staurolite, ilmenite, magnetite, garnet, quartz, epidote, olivine and alteration products as inclusions, which comprises subjecting a pulp of such an ore to an initial blunging treatment in the presence of a soluble fluosilicate-forming substance, partially neutralizing the acidified particle surfaces by introducing a caustic into the pulp, subjecting said pulp to a bulk froth flotation action in the presence of a fatty acid collector to concentrate the chrome-containing constituents of the pulp, refloating the concentrate of the treatment in a plurality of cleaning actions while increasing the acidity of the pulp in each such refloating action through the introduction of a mineral acid therein, whereby to selectively reject different minerals of the pulp, recovering a purified chromite concentrate as a final product of the treatment, and recovering a garnet residue from one of said treatment stages as another final product of the treatment.

3. A selective froth flotation process for the treatment of chromite ores having low grade chrome spinels, zircon, staurolite, ilmenite, magnetite, garnet, quartz, epidote, olivine and alteration products as inclusions, which comprises subjecting a pulp of such an ore to an initial blunging treatment in the presence of a soluble fluosilicate-forming substance, partially neutralizing the acidified particle surfaces by introducing a caustic into the pulp, subjecting said pulp to a bulk froth flotation action in the presence of a fatty acid collector to concentrate the chrome-containing constituents while rejecting quartz, epidote, olivine and alteration products, increasing the acidity of the pulp by entering a quantity of mineral acid into the froth concentrate product so formed, refloating said concentrate in a second froth flotation action to reject garnet, entering additional mineral acid into the froth concentrate of said second action, refloating said second concentrate in a third froth flotation action to reject magnetite, ilmenite, staurolite, zircon and low grade chrome

spinels, and collecting purified chromite as a final froth concentrate of the treatment.

4. A selective froth flotation process for the treatment of chromite ores having low grade chrome spinels, zircon, staurolite, ilmenite, magnetite, garnet, quartz, epidote, olivine and alteration products as inclusions, which comprises subjecting a pulp of such an ore to an initial blunging treatment in the presence of a soluble fluosilicate-forming substance, partially neutralizing the acidified particle surfaces by introducing a caustic into the pulp, increasing the acidity of the pulp by introducing some mineral acid therein, subjecting said pulp to a froth flotation action in the presence of a fatty acid collector to concentrate the chrome-containing constituents while rejecting quartz, epidote, olivine and alteration products, entering additional mineral acid into the froth concentrate product so formed, subjecting said concentrate product to another froth flotation treatment to collect the other chrome-containing constituents while rejecting garnet, removing the reject garnet product as a concentrate of the treatment, entering additional mineral acid into the froth concentrate of said second action and refloating said second concentrate in a third froth flotation action in which at least one of the chrome-containing constituents consisting of magnetite, ilmenite, staurolite, zircon and low grade spinels is rejected.

ARTHUR J. WEINIG.

#### REFERENCES CITED

35 The following references are of record in the file of this patent:

#### UNITED STATES PATENTS

| Number       | Name       | Date           |
|--------------|------------|----------------|
| 40 1,972,588 | Hansen     | Sept. 4, 1934  |
| 1,986,816    | Hallestrom | Jan. 8, 1935   |
| 2,014,404    | Weed       | Sept. 17, 1935 |
| 2,125,631    | Gutzeit    | Aug. 2, 1938   |

#### OTHER REFERENCES

45 Conditioning Surfaces for Flotation, by Norman & Ralston in Mining Technology, May 1939, T. P. 1074, pages 1, 2, 3, 4, 5, 11, 12, 13, 15, 16.

50 Control of the Souring Operation, by B. H. Gilmore, Special Bulletin, February 1931, Laundry Owners, National Asso., pages 3 and 4, copy in 8-137.